# EUROPEAN PATENT SPECIFICATION

(11) **EP 0 730 695 B1**
(45) Date of publication and mention of the grant of the patent: **28.01.1998**
(21) Application number: 95902841.6
(22) Date of filing: 25.11.1994
(51) Int. Cl.: E04B 1/94

(54) **GAP SEAL**
FUGENDICHTUNG
JOINTS DE DILATATION POUR ESPACE VIDE

(30) Priority: 26.11.1993 GB 9324344
(43) Date of publication of application: 11.09.1996
(73) Proprietor: BTR plc, London SW1P 2PL (GB)
(72) Inventor: GANENDRAN, Arasapillai N., Swadlincote, Derby DE11 0OX (GB)
(74) Representative: Sparrow, Alvar Alfred
(86) International application number: GB9402588
(87) International publication number: WO9514828

(56) References cited:
- EP-A- 0 153 564
- EP-A- 0 312 937
- EP-A- 0 400 402
- FR-A- 2 299 045
- US-A- 3 566 541
- DATABASE WPI, Week 8718, Derwent Publications Ltd., London, GB; AN 87-127154 & JP,A,62 070 478 (SUMITOMO) 31 March 1987

## Description

This invention relates to gap seals, especially to seals for gaps between structural elements such as panels in building structures.

Gaps at the junction of structural panels, such as walls, ceilings and floors of buildings, frequently are provided to allow for small movements between the panels.

The present invention provides a seal or joint for installation in such gaps, and which accommodates variation in the size of the gap and changes in the gap size resulting from movement of the panels, for instance by expansion or contraction or lateral movement of one or more adjoining panels. Such seals are sometimes referred to as expansion joints. Furthermore, the seal or joint of this invention also provides a fire-resistant barrier in fire conditions and additionally may confer thermal and/or acoustic and/or moisture insulation.

In US-A-3566541 issued in 1971, there is described a fire-protective barrier for installation in structural gaps, which barrier consists of an assembly of at least two discrete components, namely a soft compressible mechanical gasket of resilient flexible material typified by neoprene plastic, optionally having an elongate cavity or hollow, assembled with one or more strips or masses of intumescent material.

In FR-A-2299045 published in 1976, there is described a fire-proofing sealing element consisting of a flexible impervious tube, the tubular hollow of which is filled with aqueous alkali metal silicate solution or gel which produces a silicate foam mass when subjected to fire conditions.

Both of these prior proposals require an assembly of a flexible component and an intumescent or foamable component. In contrast, the present invention provides a one-piece fire-resistant flexible resiliently compressible gap seal having inherent intumescence.

The seal of the present invention comprises a flexible resiliently radially compressible tube formed of a composition based mainly on a blend of elastomeric material and intumescent material, i e the proportions of elastomeric material and intumescent material are substantially greater than the proportion of any additional ingredient present in the composition.

Preferred additional ingredients in the composition include a fire-retardant agent and/or a fusible inorganic binder.

Other suitable ingredients include a reinforcing filler and/or a light-weight filler.

One or more additional ingredients, such as those known for use in elastomeric compositions, may also be present.

The tube may be produced in long lengths, for example by extrusion, for cutting to lengths required for the gap to be sealed.

If desired, the seal may comprise a laminate of the composition with one or more layers of other material.

The elastomeric material provides a binder for the other composition ingredients. Suitably, it may be a synthetic rubber. Preferably it is curable at a temperature lower than that at which the intumescent material commences to intumesce. A preferred elastomeric material is epdm.

A suitable intumescent material is expandable graphite material. Such material usually comprises chemically-treated graphite which commences to expand by several times its original volume, e g 100-200 times, when heated above a critical temperature, e g about 190°C. Examples of expandable graphite materials are those available under the trade name 'CALLOTEK', for instance 'CALLOTEK 100' or 'CALLOTEK 500'. Preferably, the composition contains a high proportion of intumescent material. For instance, the ratio of intumescent material to elastomeric material may be at least 1:1 by weight.

The fire-retardant agent suitably is an ablative material. A preferred fire-retardant agent is alumina trihydrate. It is found that alumina trihydrate also enables an increase in the temperature employed for curing the elastomeric material in the composition without premature activation of the intumescent material.

The fusible inorganic binder is a material which is capable of melting and resolidifying at elevated temperatures such as fire temperatures. A preferred fusible material comprises glass particles. Preferably the fusible material comprises a mixture of particles having different melting points, suitably commencing at about 200°C. Such a particle mixture may melt progressively over a temperature range of about 200°C to 900°C, for instance about 350°C to 700°C. The material then resolidifies above the melting temperature. For instance, resolidification may commence at a temperature above about 700°C or above about 900°C to form a crystalline solid. In doing so, it acts as a binder for maintenance of stability of the seal in fire conditions. Examples of suitable fusible glass particles are those available under the trade name "Ceepree" ex ICI/Brunner Mond & Company.

A suitable reinforcing filler for the composition is carbon black.

A suitable light-weight filler may be, for instance, hollow microspheres such as polymeric microballoons. The polymeric microballoons preferably are of a resilient material, for example epdm. Suitable resilient microballoons are those obtainable under the trade name 'EXPANCEL'.

Other ingredients may be selected from, for example, curatives, accelerators, processing aids, anti-ageing agents, fungicides, pigments, fibre reinforcements, etc.

By way of example only, a composition suitable for a seal or joint according to the invention may have the following formulation:-

| Ingredients | Parts by weight |
|---|---|
| Elastomer (epdm) | 100 |
| Intumescent agent (expandable graphite) | 100-200 |
| Fire-retardant agent (alumina trihydrate) | 20 |
| Fusible inorganic particles ('Ceepree') | 10 |
| Filler (carbon black) | 30 |
| Light-weight filler ('EXPANCEL') | 10 |
| Other ingredient(s) | 5 |

The composition ingredients may be blended by conventional techniques.

The tubular form of the seal may be produced by, for instance, extrusion of the composition.

The composition may be subjected to elastomer-curing conditions in its tubular form. The cure temperature preferably should be below that at which the intumescent material would start to intumesce. An example of a suitable cure temperature is about 150°C.

The seal is suitable for indoor and outdoor applications.

Suitably the external diameter of the seal in its uncompressed state is greater than the width of the gap to be sealed, so that the seal is held in compressed state in the gap. A preferred level of compression of the seal in the gap is at least about 20% of the uncompressed seal diameter.

The tubular wall thickness of the seal preferably should be such that, when the seal is subjected to fire conditions which degrade the elastomeric material, the composition expands intumescently into the hollow of the tube and across the gap to maintain or increase the barrier effect of the seal, and thereby prevents traverse of flame, smoke and other hazardous fire products.

The ratio of the tubular wall thickness to the uncompressed seal external diameter may be in the range of, for instance, 0.08:1 to 0.5:1. Preferably the ratio is at least about 0.1:1.

By way of example only, dimensions and corresponding compressions of the seal are given below, in which:-
W = gap width;
CD = compressed external diameter of the seal along the depth of the gap;
UD = external diameter of the seal in its normal uncompressed state;
C = compression of the seal widthwise of the gap.

| CD : W | W : UD | C (%) |
|---|---|---|
| 1:1 | 0.785:1 | 21.5 |
| 2:1 | 0.523:1 | 47.7 |
| 3:1 | 0.393:1 | 60.7 |
| 4:1 | 0.314:1 | 68.6 |
| 5:1 | 0.262:1 | 73.8 |
| 15:1 | 0.098:1 | 90.2 |

The cross-sectional outer shape of the tubular wall of the seal (i e in a plane perpendicular to the longitudinal axis of the tube) may be of any shape suitable for fitting the seal into the gap to be sealed. Typically, the tubular wall of the seal, in its normal uncompressed state, has a substantially circular cross-sectional surface shape, but alternatively it may have, for instance, an elliptical or a polygonal outer surface shape.

Optionally, the seal may be provided with one or more longitudinal slits in the wall, extending from the external surface thereof, to facilitate compression for insertion into a gap. One such slit may penetrate completely through the wall if desired, and in that case the seal preferably should be located in the gap such that the slit is not exposed.

The names 'CALLOTEK', 'Ceepree' and 'EXPANCEL' are proprietary trade names.

## Claims

1. Seal for a gap between structural elements, which provides a fire-resistant barrier in fire conditions and which comprises intumescent material and a flexible compressible hollow gasket of resilient material, characterised in that the seal comprises a flexible resiliently radially compressible tube formed of a composition based mainly on a blend of elastomeric material and intumescent material.

2. Seal according to Claim 1 wherein the intumescent material comprises expandable graphite.

3. Seal according to Claim 1 or 2 wherein the ratio of intumescent material to elastomeric material is at least 1:1 by weight.

4. Seal according to any of the preceding Claims wherein the elastomeric material comprises epdm.

5. Seal according to any of the preceding Claims wherein the composition comprises also a fire-retardant agent.

6. Seal according to Claim 5 wherein the fire-retardant agent comprises alumina trihydrate.

7. Seal according to any of the preceding Claims wherein the composition comprises also a fusible inorganic binder being a material which is capable of melting and re-solidifying at normal fire temperatures.

8. Seal according to Claim 7 wherein the fusible inorganic binder comprises a mixture of glass particles having various melting points.

9. Seal according to any of the preceding Claims wherein the composition comprises also one or more fillers.

10. Seal according to Claim 9 wherein the composition contains light-weight filler being resilient microballoons of polymeric material.

11. Seal according to any of the preceding Claims having a tubular form produced by extrusion.

12. Seal according to any of the preceding Claims wherein the ratio of the tubular wall thickness to the external diameter of the seal in its uncompressed state is in the range 0.08:1 to 0.5:1.

13. Seal according to Claim 12 wherein said ratio is at least 0.1:1.

14. Seal according to any of the preceding Claims which, when present in a gap as a gap seal between structural elements, is under radial compression by at least about 20% of the uncompressed seal diameter.

15. Seal according to any of the preceding Claims having one or more longitudinal slits in the tubular wall, extending from the outer surface of the wall.

## Patentansprüche

1. Dichtung für eine Fuge zwischen Bauelementen, die eine feuerfeste Barriere in Feuerbedingungen liefert und die anschwellendes Material und ein flexibles, zusammendrückbares, hohles Dichtungselement aus federndem Material umfaßt,
dadurch **gekennzeichnet,**
daß die Dichtung ein flexibles, federnd radial zusammendrückbares Rohr umfaßt, das aus einer Zusammensetzung gebildet ist, die hauptsächlich auf einer Mischung aus elastomerem Material und anschwellendem Material beruht.

2. Dichtung nach Anspruch 1, wobei das anschwellende Material ausdehnbares Graphit umfaßt.

3. Dichtung nach Anspruch 1 oder 2, wobei das Gewichtsverhältnis von anschwellendem Material zu elastomerem Material zumindest 1:1 beträgt.

4. Dichtung nach einem der vorhergehenden Ansprüche, wobei das elastomere Material EPDM umfaßt.

5. Dichtung nach einem der vorhergehenden Ansprüche, wobei die Zusammensetzung ebenso ein feuerhemmendes Mittel umfaßt.

6. Dichtung nach Anspruch 5, wobei das feuerhemmende Mittel Aluminiumoxidtrihydrat umfaßt.

7. Dichtung nach einem der vorhergehenden Ansprüche, wobei die Zusammensetzung ebenso ein schmelzbares, anorganisches Bindemittel umfaßt, das ein Material ist, das in der Lage ist, bei normalen Feuertemperaturen zu schmelzen und sich wieder zu verfestigen.

8. Dichtung nach Anspruch 7, wobei das schmelzbare, anorganische Bindemittel eine Mischung aus Glaspartikeln mit verschiedenen Schmelzpunkten umfaßt.

9. Dichtung nach einem der vorhergehenden Ansprüche, wobei die Zusammensetzung ebenso einen oder mehrere Füllstoffe umfaßt.

10. Dichtung nach Anspruch 9, wobei die Zusammensetzung Leichtgewichtsfüllstoff enthält, der aus federnden Mikroballonen aus polymerem Material besteht.

11. Dichtung nach einem der vorhergehenden Ansprüche, die eine durch Extrudieren erzeugte Rohrform aufweist.

12. Dichtung nach einem der vorhergehenden Ansprüche, wobei das Verhältnis der Rohrwanddicke zum Außendurchmesser der Dichtung in ihrem nicht zusammengedrückten Zustand im Bereich von 0,08:1 bis 0,5:1 liegt.

13. Dichtung nach Anspruch 12, wobei das Verhältnis zumindest 0,1:1 beträgt.

14. Dichtung nach einem der vorhergehenden Ansprüche, die, wenn sie in eine Fuge als eine Fugendichtung zwischen Bauelementen vorhanden ist, sich unter radialer Zusammendrückung um zumindest ungefähr 20 % des nicht zusammengedrückten Dichtungsdurchmessers befindet.

15. Dichtung nach einem der vorhergehenden Ansprüche, die einen oder mehrere Längsschlitze in der Rohrwand aufweist, die sich von der äußeren Oberfläche der Wand erstrecken.

## Revendications

1. Joint d'étanchéité pour un espace entre des éléments de construction, qui constitue une barrière résistante au feu en cas d'incendie, et qui comprend une matière intumescente et un joint creux, compressible et flexible en une matière élastique, caractérisé en ce qu'il comprend un tube flexible élastiquement et radialement compressible, en une composition essentiellement à base d'un mélange d'une matière élastomère et d'une matière intumescente.

2. Joint d'étanchéité selon la revendication 1, dans lequel la matière intumescente comprend du graphite dilatable.

3. Joint d'étanchéité selon la revendication 1 ou 2, dans lequel le rapport de la matière intumescente à la matière élastomère est au moins de 1 : 1 en poids.

4. Joint d'étanchéité selon l'une quelconque des revendications précédentes, dans lequel la matière élastomère comprend de l'epdm.

5. Joint d'étanchéité selon l'une quelconque des revendications précédentes, dans lequel la composition comprend en outre un agent ignifuge.

6. Joint d'étanchéité selon la revendication 5, dans lequel l'agent ignifuge comprend du trihydrate d'alumine.

7. Joint d'étanchéité selon l'une quelconque des revendications précédentes, dans lequel la composition comprend de plus un liant inorganique fusible, qui est une matière propre à fondre et à se resolidifier à des températures normales d'incendie.

8. Joint d'étanchéité selon la revendication 7, dans lequel le liant inorganique fusible comprend un mélange de particules de verre ayant divers points de fusion.

9. Joint d'étanchéité selon l'une quelconque des revendications précédentes, dans lequel la composition comprend également une ou plusieurs charges.

10. Joint d'étanchéité selon la revendication 9, dans lequel la composition comprend une charge légère, consistant en des microbilles élastiques en une matière polymère.

11. Joint d'étanchéité selon l'une quelconque des revendications précédentes, qui a une forme tubulaire obtenue par extrusion.

12. Joint d'étanchéité selon l'une quelconque des revendications précédentes, dans lequel le rapport de l'épaisseur de la paroi tubulaire au diamètre extérieur du joint d'étanchéité, à l'état non comprimé, est compris dans la plage de 0,08 : 1 à 0,5 : 1.

13. Joint d'étanchéité selon la revendication 12, dans lequel ledit rapport est d'au moins 0,1 : 1.

14. Joint d'étanchéité selon l'une quelconque des revendications précédentes, qui, lorsqu'il est présent dans un espace entre des éléments de construction en tant que joint d'étanchéité, est soumis à une compression radiale représentant au moins 20 % du diamètre du joint d'étanchéité à l'état non comprimé.

15. Joint d'étanchéité selon l'une quelconque des revendications précédentes, comportant une ou plusieurs fentes longitudinales dans la paroi tubulaire, qui s'étendent à partir de la surface extérieure de la paroi.
